

# UNITED STATES PATENT OFFICE.

TURNER D. BOTTOME, OF HOOSICK, NEW YORK.

## ANTIFRICTION ALLOY.

SPECIFICATION forming part of Letters Patent No. 484,084, dated October 11, 1892.

Application filed December 29, 1891. Serial No. 416,411. (No specimens.)

*To all whom it may concern:*

Be it known that I, TURNER D. BOTTOME, a citizen of the United States, and a resident of Hoosick, in the county of Rensselaer and State of New York, have invented certain new and useful Improvements in Antifriction Alloys, of which the following is a specification.

This invention relates to that class of white-metal alloys known more particularly under the name of "antifriction-bearing metals."

In mechanics a very exact line is drawn between the various kinds of bearings, and they are divided chiefly into two large groups—namely, red brass or bronze and the so-called "white-metals" or "Babbitt" bearings. The red-brass bearings are distinguished by their great hardness and power of resistance, but have a very high melting-point. Hence their use is limited by reason of the cost and mechanical labor involved in order to make a good bearing from them. White-metals, on the other hand, have a moderately-low melting-point, so that a worn-out bearing can be remelted and readily replaced with a new one

at a small expense. Furthermore, being reasonably soft and compressible, they do not injure the journals under any circumstances.

White-metal alloys for bearings are divided into two general classes, one a cheap grade, which consists largely of lead which forms the basis, and in order to harden it a proportion of antimony is alloyed therewith in varying quantity, and sometimes a small quantity of copper or tin or both are added in order to produce certain qualities, such as rendering the alloy harder or more fusible. For the latter quality a little bismuth is often added. A few of the cheap mixtures have zinc as a basis, but their use is limited. The general

run of antifriction alloys, however, are designated as "high-grade Babbitts." They are more costly and are better adapted for their purposes than the cheaper classes as they are at present prepared. The basis of these high-grade antifriction metals is essentially metallic tin, one of the most familiar of these alloys being composed of eighty-five parts tin, ten of antimony, and five of copper, yet the composition varies considerably, and other metals are sometimes added for imparting some special property. All of these alloys may be said to be more or less suitable for bearings,

some of them being specially adapted for slow-moving journals heavily loaded, while others are better adapted for light-running high-speed machinery. There is a gap between these two extremes that hitherto has only been filled with the class of red-brass bearings, among which aluminum bronze and tempered copper stand at the head as examples of wearing quality and great power of resistance.

Many of the alloys in practical use that give more or less satisfaction to the users as far as their wearing quality is concerned still have the disagreeable property of contracting upon solidification of the melted metal, thus necessitating the labor of scraping a fit before the bearing can be used, and many of the metals do fairly well if given a liberal supply of best quality lubricating-oil, which, however, is an expensive method of keeping a bearing in good order. Another feature inherent in all of the white antifriction metals is the fault of wearing away rapidly under load, coloring the oil black, and often becoming so hot as to actually fuse.

This invention has for its object the production of a white-metal bearing suitable for heavily-loaded journals subjected to high speeds and as a successful substitute for the class of red-brass bearings.

Another object is the production of an alloy that will run cool with a minimum supply of oil of fair quality and yet wear away but slowly, having the further valuable property of neither contracting nor expanding upon solidification of the melted metal, yet retaining perfect fluidity when melted and capable of pouring to make any possible form of box or bearing.

The last and most important object of this invention is the cheapness with which it can be prepared, enabling it successfully to compete not only with the high-grade antifriction alloys, but also with the cheaper classes, thus placing it within reach of every one that has occasion to use bearing metals.

These objects are obtained in the following manner: First, an alloy is prepared, consisting of lead, from three to sixteen parts to one part of tin and from one to ten parts of antimony. This alloy forms a basis for the finished metal. Used alone it has no special advantage over any other alloy of its class, it

belonging, as may be readily observed, to the cheap class. In order that this cheap alloy will attain its maximum and valuable properties it must be tempered. The chief feature and merit of this invention lie in the discovery I have made that the metal magnesium added to any of the ordinary bearing metals, even in very small quantities, imparts to them remarkable properties. The proportion of this metal in the finished alloy may vary considerably; but as a rule an alloy containing from one to ten parts of magnesium to one thousand of the basis or lead alloy described produces the best-quality bearings. Magnesium is a very light metal. Its specific gravity is 1.7, being seven times lighter than lead. It has the property of burning with a most intense white light when the pure metal is heated to redness in the air, and, like the metal aluminium, it is of great tensile strength and toughness, which it imparts to its alloys. It has the property of forming alloys with most of the base metals, including lead, antimony, and tin. These metals used together and alloyed even with a minute quantity of magnesium impart properties of a totally-dissimilar character from those as ordinarily known. In fact, a new metal has been produced, having properties belonging to no other metal or alloy hitherto known to science. These properties are hardness, toughness, great resistance to compression, malleability, fusibility, great cohesiveness, imparting a property-resisting wear by attrition, and, lastly, the long-sought for property of neither contracting nor expanding upon solidification. The above-named properties account for the great and decided superiority of this metal over all others of its class for antifriction purposes. In order, therefore, to "temper" the cheap lead alloy it is necessary to introduce a certain quantity of magnesium. As ordinarily metals are introduced to form alloys by simply putting them in the melted mixture, the extreme lightness of this metal would cause it to float on the surface, and thus take fire. Hence another mode must be used. It is for this reason that I prefer to form a special "tempering-alloy" of known composition rich in magnesium. Preferably this tempering-alloy is prepared by melting

about nine parts of tin together with one part of magnesium in a closed vessel free from oxygen and preferably in an atmosphere of hydrogen. However, the tempering-alloy may be prepared with lead or with a small quantity of the base alloy direct. I do not limit myself to any particular process or method of forming it nor to any specified proportions of metal in the said tempering-alloy. So long as the metal magnesium is present it is sufficient for the purpose, and it matters but little how it gets into the finished composition. The tempering-alloy thus prepared is then added to the base alloy (previously melted to fluidity) by forcing the tempering below the surface of the molten metal. Certain other metals may be introduced into the alloy, but apparently with no particular advantages over the composition as herein given. I do not limit the scope of the invention merely to an alloy of lead, antimony, and tin with a small content of magnesium, but include other alloys of this general class, and especially the white antifriction metals as a generic class when such contain a sufficient content of magnesium to alter their properties in such a way as to make them better adapted as bearing metals.

Having thus described the characteristics peculiar to antifriction alloys containing magnesium, what I claim as my invention is as follows:

1. An antifriction alloy consisting of lead, antimony, tin, and magnesium, as described.
2. An antifriction alloy consisting of eight hundred parts of lead, one hundred and fifty parts of antimony, fifty parts of tin, and two parts of magnesium.

3. An antifriction alloy consisting of three to sixteen parts of lead, one to ten parts of antimony, one part of tin, more or less, and one to ten parts of magnesium to each one thousand parts of first-named metals when mixed together, substantially as described.

Signed at Hoosick, in the county of Rensselaer and State of New York, this 26th day of December, A. D. 1891.

TURNER D. BOTTOOME.

Witnesses:

A. H. HAWKS,  
J. S. BALL.